

Patented June 15, 1954

2,681,265

# UNITED STATES PATENT OFFICE

2,681,265

## SPINNING ARTIFICIAL FILAMENTS

Howard M. Hoxie, Chester, Pa., assignor to American Viscose Corporation, Wilmington, Del., a corporation of Delaware

No Drawing. Application November 27, 1948,  
Serial No. 62,413

8 Claims. (Cl. 18—54)

1

This invention relates to the production of synthetic filaments or yarns comprising acrylonitrile polymers.

The patent literature contains statements to the effect that acrylonitrile polymers containing at least 85% by weight acrylonitrile in the polymer molecule can be formed into synthetic filaments or yarns by extruding a dimethyl formamide solution of the polymer into water at a temperature of 70° C., and stretching the filaments or yarns thus obtained to 6.3 times their original length.

In actual practice, it has been found to be impossible to obtain useful filaments or yarns by spinning the dimethyl formamide solutions into a bath consisting of water, regardless of variations in such factors as immersion length, bath temperature, spinning speed, jet design, or filament size. The filaments obtained by spinning the solutions into a bath consisting of water are extremely weak, fragile, and brittle, and are practically inextensible. Such filaments or yarns comprise areas which are too completely coagulated for stretching, and areas which are incompletely coagulated, the more completely coagulated areas occurring, generally, at the surface of the filament, which thus comprises a layer of coagulated polymer surrounding a plastic core. Evidently, this condition of the filaments obtained by spinning the dimethyl formamide solutions into a bath consisting of water is due to differences between the rate of diffusion (or extraction) of the dimethyl formamide from the interior of the fiber outwardly, and the rate of diffusion of the coagulating liquid inwardly, whereby diffusion of the spinning solvent out of the fiber is prevented or hampered by the coagulated layer formed initially at the surface of the filament. Whatever may be the explanation of the difficulty, it is a fact that when the solutions are spun into water, the filaments withdrawn from the bath are not capable of accepting sufficient stretch to effect appreciable molecular orientation without rupture. In order to obtain useful filaments from the solutions by the wet spinning method, it has been necessary to employ organic solvents such as isopropanol, glycerol, or aqueous salt solutions, such as aqueous solutions of calcium chloride, as the coagulating liquid. All such liquids entail troublesome problems of coagulating bath regeneration and solvent recovery.

It is, therefore, an object of this invention to provide a new method of producing filaments and yarns from solutions of the acrylonitrile polymers in dimethyl formamide by a wet spin-

2

ning procedure, whereby homogeneous filaments capable of being stretched without rupture are formed in the bath. Another object is to provide such a method in accordance with which the spinning is performed at room temperature. A further object is to provide such a method wherein regeneration of the coagulating bath and recovery of the spinning solvent are simplified.

10 These and other objects are achieved by the present invention, in accordance with which solutions of the acrylonitrile polymers in dimethyl formamide are spun into a coagulating bath consisting of a mixture of water and dimethyl formamide containing from 35 to 80% by volume of dimethyl formamide, at room temperature. The filaments thus formed are withdrawn from the coagulating bath after an immersion distance of from 1 to 40 inches, and given a stretch of from 200 to 300%. The filaments withdrawn from the bath are coagulated so that they possess sufficient plasticity to permit extension thereof under stretching, without rupture. It is known that stretching of the acrylonitrile polymer filaments effects an improvement in the physical properties such as tenacity and resilience. While it has been stated in the patent literature that acrylonitrile polymer yarns produced by wet spinning a dimethyl formamide solution of the polymer can be stretched at any time, after their formation actually in the usual practice the stretching is performed after the filaments have been withdrawn from the coagulating bath and before washing to remove the remaining solvent. The filaments produced by the present method are generally stretched by 200 to 300% after they are withdrawn from the dimethyl formamide-water spinning bath prior to washing thereof. This stretching can be accomplished at room temperature by passing the filaments, as they advance from the coagulating bath, between rollers or godets rotating at different peripheral speeds. Alternately, while the filaments are passing between stretching rollers or godets they may be caused to contact a heated stationary pin or to pass through a heated inert medium such as air, mineral oil, or glycerol.

15 The acrylonitrile polymer which is dissolved in dimethyl formamide and spun into a coagulating bath consisting of a water-dimethyl formamide mixture containing from 35 to 80 volume per cent of dimethyl formamide in accordance with this invention may be polyacrylonitrile, or it may be a copolymer or interpolymer in which acrylonitrile is copolymerized or interpolymerized with another polymerizable substance containing

3

the group  $>\text{C}=\text{C}<$ , such as for example, 2-vinyl pyridine, vinyl acetate, vinyl chloride, acrylic acid and its esters, styrene, isobutene, and butadiene, as well as other vinyl and acrylic compounds, and other olefin or diolefin hydrocarbons. The coagulating baths of the present invention are particularly useful in the spinning of dimethyl formamide solutions of acrylonitrile polymers containing at least 65% by weight acrylonitrile in the polymer molecule and having a molecular weight of 15,000 to 250,000 as determined by specific viscosity data using the Staudinger equation, since those polymers are suitable for the production of filaments and yarns which may be used for general textile purposes.

The advantages of the method of this invention are numerous and important. Spinning can be performed at room temperature, thus eliminating the need for means for heating the bath. Once the spinning operation has been initiated the only expedient required in order to maintain the composition of the spinning bath constant is the periodical or continuous addition of the calculated amounts of plain water, so that expensive bath recirculating and regenerating systems are entirely avoided. In addition, the solvent recovery procedure is simple since in order to recover the solvent, it is only necessary to distill off the water, which can be accomplished rapidly and at comparatively little ex-

|                                   | Filaments | Denier | Tensile Strength, gms./denier | Extensibility, percent |
|-----------------------------------|-----------|--------|-------------------------------|------------------------|
| Before Relaxation                 | 44        | 54     | 4.9                           | 8                      |
| After Relaxation in Boiling Water | 44        | 62     | 4.2                           | 20                     |

pense. Further advantages are that the coagulating bath is non-inflammable, non-volatile, and relatively non-toxic.

In the practice of this invention, the concentration of dimethyl formamide in the bath must be maintained at from 35 to 80% by volume throughout the entire spinning operation.

This requires the addition of only small amounts of water. In the case of other spinning baths, for example, glycerol, the presence of more than a small amount, not over 20%, of dimethyl formamide is detrimental and results in breaking of the filaments at the jet and excessively weak yarns. In order to keep the concentration of dimethyl formamide introduced during spinning into a glycerol precipitating bath at or below the comparatively low critical value for satisfactory spinning, it is necessary to add substantial amounts of the expensive glycerol to the bath. Thus, for each liter of dimethyl formamide pumped into the bath as dope, it is necessary to add four liters of glycerol in order to prevent increase in the dimethyl formamide concentration above 20%. In contrast to this, when the spinning bath comprises a mixture of, say, 67% dimethyl formamide and 33% water, amounts of dimethyl formamide greater than are introduced as dope do not have to be added, and it is necessary to add only  $\frac{1}{2}$  a liter of water to the bath, for each liter of dimethyl formamide pumped in as dope, in order to maintain the necessary bath composition.

The filaments or yarns obtained by the present method compare favorably with, and in many cases are superior to, the yarns which can be obtained by spinning the solutions of the acrylonitrile polymers into organic solvents such as glycerol, or into salt solutions.

The acrylonitrile polymers which are formed into filaments or yarns in accordance with the invention may be produced by any suitable polymerization procedure, e. g., by emulsion, suspension, bulk, or solution polymerization procedures. The following examples are illustrative of pre-

The following examples are illustrative of preferred methods of practicing the invention, although the invention is not to be limited by the details set forth therein.

*Example I*

13% dimethyl formamide solution of a copolymer which was prepared by the solution copolymerization of acrylonitrile and 2-vinyl pyridine and which contained 15% of 2-vinyl pyridine by weight in the polymer molecule was extruded through a spinneret having 44 holes each having a diameter of 4 mils into a coagulating bath consisting of 30% water and 70% dimethyl formamide, by volume, at 23° C. After a bath travel of 9.5 inches, at a speed of 260 inches/min. the yarn was withdrawn from the bath and stretched 220% between two pairs of canted godets. The yarn was then washed with water, collected, and dried in air. It had a dry tenacity of 1.3 gms. per denier; dry extensibility, 25%. The yarn was then stretched 350% by passing it through a tube heated to 175° C. at a speed of 70 ft./min. The resulting yarn had the following characteristics:

40 The tenacity and extensibility of the final heat-stretched yarn are essentially the same as those of a yarn obtained by spinning the dimethylformamide solution into glycerol or calcium chloride solution, at elevated temperatures, in spite of the fact that, prior to the final heating and stretching step, the tensile strength of the yarn  
45 was somewhat lower than that of yarns obtained when organic solvents or salt solutions were used to effect the coagulation. The yarn produced by the present method exhibits excellent stability at high temperature, is not cemented, and can  
50 be dyed by means of wool dyes of the strong acid type, such as Wool Fast Scarlet. The yarn is substantially free from voids when examined under a microscope which magnifies the cross section 500 times.

### Example II

A 15% solution of polyacrylonitrile in dimethyl formamide was extruded through a 40-hole 3-mil jet into a bath comprising 32% water and 68% dimethyl formamide by volume. After an immersion of five inches (speed=260 in./min.) the yarn was withdrawn from the bath, stretched 200%, washed in water, and dried.

This yarn had a tensile strength of 1.2 g/d. and an extensibility of 24%. 300% stretch was applied to the yarn during its passage through a tube heated to 160° C. The tenacity of the heat-stretched yarn was 4.6 gms/denier. After relaxation in boiling water the tenacity was 3.82 gms/denier, the extensibility 13%, and the denier 74.

### Example III

A copolymer containing 17% acrylamide and 83% acrylonitrile by weight was prepared by 75 water solution polymerization. A 12% solution

of this polymer in dimethyl formamide was extruded through a 90-hole 3-mil jet into a bath comprising 55% water and 45% dimethyl formamide. After an immersion of three inches (speed=260 in./min.) the yarn was withdrawn from the bath, stretched 200%, washed, and dried. The yarn so obtained had a tenacity of 1.42 gms./denier and an extensibility of 28.3%. Passage through a tube heated to 180° C. permitted application of 400% stretch and produced a yarn of 95 denier which had a tenacity of 5.1 gms./denier and an extensibility of 8%.

Since it is obvious that some changes and modifications can be made in the above described details without departing from the nature and spirit of the invention, it is to be understood that the invention is not to be limited thereto except as defined in the appended claims.

I claim:

1. A method for the production of yarns from a solution of a fiber-forming acrylonitrile polymer containing, in the polymer molecule, at least 65% of acrylonitrile in dimethyl formamide which comprises spinning the solutions into a coagulating bath consisting essentially of a mixture of water and from 35 to 80% by volume of dimethyl formamide, withdrawing the yarn thus formed from the bath, and stretching the yarn by 200 to 300% of its length, the composition of the coagulating bath being maintained substantially constant from the beginning to the end of the spinning operation.

2. A method as in claim 1, wherein the coagulating bath consists of a mixture of water and 70% by volume of dimethyl formamide.

3. A method as in claim 1, wherein the acrylonitrile polymer is a copolymer of acrylonitrile and 2-vinyl pyridine containing 85% by weight of acrylonitrile in the polymer molecule.

4. A method as in claim 1, wherein the acrylonitrile polymer is polyacrylonitrile.

5. A method as in claim 1, wherein the acrylonitrile polymer is a copolymer of acrylonitrile and acrylamide containing 83% by weight of acrylonitrile in the polymer molecule.

6. A method as in claim 1, wherein the spinning is performed at room temperature.

7. A method as in claim 1, wherein the acrylonitrile polymer is a copolymer of acrylonitrile and vinyl acetate containing at least 65% by weight of acrylonitrile in the polymer molecule.

8. A method as in claim 1, wherein the acrylonitrile polymer is a copolymer of acrylonitrile and an acrylic acid ester containing at least 65% by weight of acrylonitrile in the polymer molecule.

References Cited in the file of this patent

UNITED STATES PATENTS

| Number    | Name           | Date          |
|-----------|----------------|---------------|
| 2,236,061 | Izard          | Mar. 25, 1941 |
| 2,360,406 | Dreyfus        | Oct. 17, 1944 |
| 2,404,714 | Latham         | July 23, 1946 |
| 2,404,723 | Merner         | July 23, 1946 |
| 2,420,565 | Rugeley et al. | May 13, 1947  |